

[54] PROCESS FOR IMPARTING TO TEXTILE MATERIALS A SOFT HANDLE USING UNSATURATED ALIPHATIC ACID AMIDES

[75] Inventors: Jörg Kern, Waldkraiburg, Fed. Rep. of Germany; Christian Guth, Basel, Switzerland

[73] Assignee: Ciba-Geigy Corporation, Ardsley, N.Y.

[21] Appl. No.: 64,659

[22] Filed: Aug. 8, 1979

[30] Foreign Application Priority Data

Aug. 18, 1978 [CH] Switzerland ..... 8788/78

[51] Int. Cl.<sup>3</sup> ..... B05D 3/02

[52] U.S. Cl. ..... 427/389; 8/495; 8/639; 252/8.8; 427/389.9; 437/392; 428/260; 428/270; 428/272

[58] Field of Search ..... 427/390 A, 390 B, 390 C, 427/390 D, 390 E, 389, 389.9, 392; 8/115.5, 128, 194, 495, 639; 260/17.4 G, 17.4 C, 8, 29.6 RW; 525/296, 426, 374, 445; 428/260, 270, 272, 274; 252/8.8

[56] References Cited

U.S. PATENT DOCUMENTS

2,718,478 9/1955 Fluck et al. ..... 427/390 B X  
3,161,679 12/1964 D'Errico et al. ..... 260/561 N  
3,822,145 7/1974 Liebowitz et al. ..... 427/390 B X  
3,992,304 11/1976 Minegishi et al. ..... 8/115.5 X  
4,182,790 1/1980 Schmidle ..... 428/260

FOREIGN PATENT DOCUMENTS

2181047 11/1973 France .

1424698 2/1976 United Kingdom .

Primary Examiner—Ronald H. Smith

Assistant Examiner—Thurman K. Page

Attorney, Agent, or Firm—John P. Spitals; Edward McC. Roberts

[57] ABSTRACT

A process for imparting to textile materials a soft handle finish is disclosed, wherein an acid amide of the formula



or a reaction product from acrylic or methacrylic acid, or the lower alkyl esters of these acids, and an amine of the formula



is used as a soft-handle agent.  $\text{R}_1$  is alkyl or alkenyl having 14 to 22 carbon atoms, and  $\text{X}$  is hydrogen or methyl.

There is preferably produced from the acid amide and commercial emulsifiers and wetting agents, in a novel composition, a concentrated high-pressure emulsion, which is diluted to give an aqueous preparation that is applied to the textile materials.

12 Claims, No Drawings

PROCESS FOR IMPARTING TO TEXTILE  
MATERIALS A SOFT HANDLE USING  
UNSATURATED ALIPHATIC ACID AMIDES

The present invention relates to a process for imparting to textile materials a soft handle, in which process there is used an acid amide of the formula



wherein  $\text{R}_1$  is alkenyl or preferably alkyl having 14 to 22 carbon atoms, and  $\text{X}$  is hydrogen or methyl.

The acid amides of the formula (1) are known per se and are produced by known methods. Thus, for example, the U.S. Pat. No. 3,161,679 describes N-(octadecyl)-acrylic acid amide, its use as an intermediate for wetting agents and detergents, and its production according to U.S. Pat. No. 2,573,673 from octadec-1-ene and acrylonitrile in the presence of sulfuric acid using the so-called Ritter reaction.

It is possible to use according to the present invention, instead of pure acid amides of the formula (1), which are produced for example according to the U.S. Pat. No. 2,573,673, also reaction products from acrylic acid or methacrylic acid, or the lower alkyl esters of these acids, and the amine of the formula



wherein  $\text{R}_1$  has the given meanings. The lower alkyl groups of the acrylic or methacrylic esters, from which the reaction products are obtained, contain as a rule 1 to 4 carbon atoms. Commercial reaction products of this type usually contain 50 to 80 percent by weight of the acid amide of the formula (1) as principal product and 20 to 50 percent by weight of a mixture of the  $\beta$ -aminocarboxylic acid ester of the formula



and the  $\beta$ -aminocarboxylic acid amide of the formula



or a mixture of the  $\beta$ -aminocarboxylic acid of the formula



and the  $\beta$ -aminocarboxylic acid amide of the formula (4), wherein  $\text{R}_1$  is alkenyl or alkyl having 14 to 22 carbon atoms,  $\text{R}_2$  is alkyl having 1 to 4 carbon atoms, and  $\text{X}$  is hydrogen or methyl. Preferably,  $\text{R}_1$  is alkyl having 14 to 22 carbon atoms.

The subject matter of the invention is therefore a process for imparting to textile materials a soft handle, which process comprises applying to these materials an aqueous preparation containing at least one reaction product of the type defined or preferably an acid amide of the formula (1), and subsequently drying the material.

Further subject matter of the invention is the aqueous preparation for carrying out the process, which preparation contains, in addition to the acid amide of the formula (1) or to the reaction product, an emulsifier and optionally a wetting agent. A concentrated composition which is in the form of a concentrated emulsion or dispersion, and which contains, in addition to the acid amide of the formula (1) or to the reaction product, an

emulsifier and optionally a wetting agent, and from which the aqueous preparation is obtained by dilution with water, likewise forms subject matter of the present invention. The same applies also to the textile material to which has been imparted a soft feel by the process according to the invention.

Preferred acid amides contained in the preparation used according to the invention correspond to the formula



or particularly to the formula



wherein  $\text{R}_3$  is alkyl having 16 to 22 carbon atoms, and  $\text{X}$  has the meaning already defined.

The acid amide of particular interest is N-(octadecyl)-acrylic acid amide.

Also suitable however are commercial mixtures of the acid amides or of the reaction products, in which  $\text{R}_1$  in the formulae (1) to (5) is various alkenyl and/or alkyl groups which have 14 to 22 carbon atoms and which are derived from mixtures of fatty acids, such as are present in vegetable or animal oils and fats, especially in tallow fat.

The aqueous diluted preparation with which the textile materials are treated according to the invention contains in general 0.1 to 0.5 percent by weight, relative to the dry textile material to be treated, of the acid amide of the formula (1) or of the reaction product.

As already indicated, the preparation according to the invention is in the form of an aqueous emulsion or dispersion. For this purpose, it contains, in addition to the acid amide of the formula (1) or to the reaction product, at least one commercial emulsifier, and as a rule at least one commercial wetting agent.

Examples of commercial emulsifiers which may be mentioned are inter alia: reaction products of a fatty acid with an alkanolamine or with a polyalkylenepolyamine, the fatty acid preferably having 8 to 18 carbon atoms, the alkanolamine preferably having 1 to 10 carbon atoms, and the polyalkylenepolyamine preferably having 2 to 5 nitrogen atoms and preferably 2 to 6 carbon atoms in the alkylene moiety. These reaction products concomitantly used as emulsifiers are optionally quaternised with a dialkyl sulfate having 1 to 4 carbon atoms in the alkyl group, or optionally further reacted with a nitrile of the acrylic acid series or with an alkylene oxide having 2 or 3 carbon atoms in the alkyl group. As examples of specific emulsifiers suitable for use in the preparation used according to the invention, there may be mentioned, inter alia, reaction products of stearic acid with diethanolamine, which optionally are quaternised with dimethyl sulfate or further reacted with acrylonitrile or with ethylene oxide.

As examples of commercial wetting agents, which preferably can be contained, in addition to the acid amide of the formula (1) and to the emulsifiers given above, in the preparation for carrying out the process according to the invention, there may be mentioned inter alia: addition products of an alkylene oxide with fatty alcohols or with alkyl phenols, preferably addition products of an ethylene oxide with fatty alcohols having 8 to 24 carbon atoms, or with alkylphenols having 10 to 18 carbon atoms, with these addition products preferably containing 3 to 20 ethylene oxide units. As an example of a specific wetting agent which can be partic-

ularly well suited for use in the preparation used according to the invention, there may be mentioned, inter alia, the ethylene oxide adduct of nonylphenol, which contains 9 ethylene oxide units in the molecule.

In the aqueous emulsion, which contains an emulsifier and optionally a wetting agent, an addition of 10 percent by weight of emulsifier and 10 percent by weight of wetting agent, relative to the content of acid amide of the formula (1) or of the reaction product, is as a rule sufficient. Thus, the diluted preparation contains 0.01 to 0.05 percent by weight of at least one emulsifier and optionally 0.01 to 0.05 percent by weight of at least one wetting agent, relative to the dry textile material to be treated.

The preparations for performing the process according to the invention in general have a pH value of 4 to 6, preferably 5 to 6, which can be adjusted if necessary by the addition of a weak acid. Both inorganic weak acids, such as boric acid, phosphoric acid and carbonic acid, and mainly weak organic acids preferably having at most 4 carbon atoms, such as oxalic acid, formic acid, acetic acid, propionic acid and butyric acid, are suitable, with acetic acid being preferred.

The emulsion is produced by melting at least one acid amide of the formula (1) or at least one reaction product from acrylic acid or methacrylic acid, or alkyl esters thereof, and the amine of the formula (2), and then adding in the course of 5 to 20 minutes, with rapid stirring, an aqueous solution which is at a temperature of at least 90° C. and which contains at least one commercial emulsifier and optionally at least one commercial wetting agent of the stated type, the pH value of this solution being adjusted with an acid of the given type, particularly acetic acid, to 4 to 6. This emulsion is then advantageously subjected to high-pressure emulsification, at for example 300 to 400 Kp, for 20 to 60 minutes. The high-pressure emulsion is then cooled to room temperature, in the process of which there is generally formed a fine dispersion. This concentrated composition contains, in a novel combination, 1 to 50, preferably 5 to 25, percent by weight of the acid amide of the formula (1) or of the reaction product from acrylic acid or methacrylic acid, or esters thereof, and the amine of the formula (2), 0.1 to 5, preferably 0.5 to 2.5, percent by weight of the emulsifier described in the foregoing, and 0 to 5, preferably 0.1 to 5, especially 0.5 to 2.5, percent by weight of the wetting agent described in the foregoing. The concentrated composition has a pH value of 4 to 6, preferably 4 to 5. The great advantage of this concentrated composition is its good stability. Even after several months of storage, the composition remains homogeneous and ready for use.

To produce the diluted preparation, which is applied to the textile materials, the concentrated emulsion described in the foregoing, preferably the high-pressure emulsion which at room temperature is as a rule in the form of a fine stable dispersion, is placed into the mixing vessel just at the moment that the emulsion is to be used, and to it is then added the 5- to 10-fold amount of water at 60° to 90° C., and the whole is subsequently stirred. Not until afterwards is the dispersion further diluted with cold water, the pH value of which has been adjusted to 4 to 6 with an acid of the given type, for example acetic acid, the degree of dilution being such that there is obtained the given concentration of acid amide or of the reaction product of 0.1 to 0.5 percent by weight, relative to the textile material to be treated, which is advantageous for application.

As textile materials to which can be imparted a soft handle by the process according to the invention, there can be used materials from natural or synthetic fibres, and also mixtures thereof, preferably mixtures of natural fibres with synthetic fibres.

The textile material can be at any stage of processing, that is to say, it can be in the form of staple fibres, continuous filaments, or fleeces, particularly however in the form of flocks, yarns, fabrics or knitted goods, or articles of clothing which have already been further processed. The textile materials can have been dyed or can have been treated with an optical brightener.

The synthetic materials treated can be both semi-synthetic textile materials, for example those made from regenerated cellulose, that is to say, rayon fibres, artificial silk, viscose or cellulose acetate; and fully-synthetic textile materials, for example those made from polyacrylonitrile, acrylonitrile copolymers, polyamide or polyester.

In the case of the textile materials made from acrylonitrile copolymers or from modacrylic fibres, the proportion of acrylonitrile is advantageously at least 50 percent by weight and preferably at least 85 percent by weight of the copolymer. Copolymers particularly suitable are those for the production of which other vinyl compounds, for example vinyl chloride, vinylidene chloride, methacrylates, acrylic amide or styrenesulfonic acid, have been used as comonomers. Suitable polyamides for producing the fibres in the textile materials are for example: poly-2-caprolactam, polyhexylmethylenediamide-adipate or poly- $\omega$ -amino-undecanoic acid, while suitable polyesters are for example: poly(ethylene glycol terephthalate) or poly-(1,4-cyclohexylenedimethylene terephthalate).

As examples of textile materials made from natural fibres there may be mentioned: sisal, line, hemp and ramie, but preferably wool and in particular cotton. Materials to which a soft handle can be imparted particularly readily by the process according to the invention are above all textile materials from cotton, wool, polyamide, polyacrylonitrile, and mixtures of wool and polyacrylonitrile, of wool and polyester and of cotton and polyester. Polyacrylonitrile yarns are particularly of interest.

According to the invention, the preparations are applied by customary processes to the textile materials. Thus, for example, the preparations can be sprayed or slop-padded onto the textile materials. Preferably, however, the textile materials are padded with the preparations or are treated therewith using the exhaust process. The application is effected at room temperature or at elevated temperatures of, for example, 30° to 100° C. for 5 to 120 minutes. The textile materials are subsequently dried at room temperature or preferably at elevated temperature, for instance at 50° to 150° C.

A particular advantage of the process according to the invention is the compatibility of the employed acid amides of the formula (1) or of the reaction products and the concomitantly used emulsifiers and optionally concomitantly used wetting agents with commercial dyes and optical brighteners. Furthermore, there occurs with many dyes, especially with basic dyes, in the dyeing of polyacrylonitrile fibres no retarding action of the acid amide of the formula (1), or of the reaction product, on the concomitantly used dye. In particular, the acid amide has no unfavourable effect on the colouring strength, shade and levelness of the dyeings obtained. This is manifested especially in dyeing with dye mix-

tures, for example in the so-called trichromic process. In a particular embodiment of the process according to the invention, it is possible to impart a soft handle to the textile materials and to simultaneously dye them, that is to say, in a single treatment stage. This single treatment stage saves the energy costs which would otherwise be necessary for imparting a soft handle in a separate stage. In order to impart a soft handle and to simultaneously dye the material, there is preferably used the aforementioned exhaust process, wherein the liquor to be applied contains, in addition to the acid amide of the formula (1) or the reaction product, an emulsifier and optionally a wetting agent, also a commercial dye suitable for the type of materials to be dyed, and optionally a commercial dyeing auxiliary. It is also possible according to the invention to impart a soft handle to brightened textile material, without the degree of whiteness of the materials being impaired as a result. The same applies also when a soft handle is imparted to the textile materials at the same time as they are being brightened.

A further advantage of the process according to the invention is that the soft-handle effects obtained are well fixed and hence as a rule are fast to fine washing. The textile materials to which has been imparted a soft handle and which are fast to fine washing can, after drying, be subsequently washed at a temperature of up to about 50° C. in a domestic washing machine of customary design, with use of a commercial fine detergent, without the excellent soft-handle effects being significantly impaired. In the case of application to hydrophilic textile materials, for example cotton sponge cloth, the soft handle is imparted to the materials without any noticeable effect on their hydrophilic properties.

Particularly advantageous also is the wide range of types of materials to which a soft handle can be successfully imparted by the process according to the invention, that is to say, the versatility of application of the process according to the invention.

In a further preferred embodiment of the process according to the invention, the acid amide of the formula (1) or the reaction product from acrylic acid or methacrylic acid, and alkyl esters thereof, with the amine of the formula (2) can be used as an agent imparting a soft handle in dry-cleaning or as a rinsing agent for rendering household linen soft. In dry-cleaning, the concentrated emulsion, preferably high-pressure emulsion, which at room temperature is usually in the form of a dispersion, is added direct, that is to say, without further dilution with water, to the organic solvent used for the cleaning operation, for example perchloroethylene. Alternatively, in the washing of textile materials in the home using the customary washing procedure, the rinsing agent for imparting a soft feel is added in the form of the aqueous preparation, obtained by dilution of the concentrated emulsion or dispersion in the manner described in the foregoing, to the last rinsing bath.

In the following production instructions and examples, 'parts' and 'percentages' are by weight.

#### PRODUCTION INSTRUCTIONS FOR EMULSIONS

A. 7.5 parts of an emulsifier consisting of a reaction product from 2 mols of diethanolamine and 1 mol of stearic acid, and also 8.75 parts of a wetting agent consisting of an addition product of 9 mols of ethylene oxide with 1 mol of nonylphenol, are dissolved in 608.75 parts of water; the solution is heated to 95° C., and the

pH value is adjusted to 4 with acetic acid. As a soft-handle agent, 75 parts of the acid amide of the formula



are melted at 95° C. To this melt at 95° C. are added in the course of 10 minutes, with rapid stirring, the acid aqueous solution of the emulsifier and wetting agent. After being stirred at 95° C. for 5 minutes, the resulting pre-emulsion is subjected for 30 minutes to high-pressure emulsification at 350 Kp. The high-pressure emulsion is then cooled to 20° C. There is thus obtained a fine dispersion which is ready for use and which is storage-stable over several months. It contains 10.7% of the acid amide of the formula (4) as soft-handle agent.

B. The procedure is carried out as described in Instruction A except that the emulsifier added consists of 7.5 parts of a reaction product from 1 mol of diethylenetriamine, 1 mol of acrylonitrile and 2 mols of stearic acid, and the soft-handle agent added consists of 75 parts of the acid amide of the formula



wherein R<sub>4</sub> denotes

- 50 to 80% of  $-(\text{CH}_2)_{17}-\text{CH}_3$
- 20 to 30% of  $-(\text{CH}_2)_{15}-\text{CH}_3$
- 5 to 15% of  $-(\text{CH}_2)_{13}-\text{CH}_3$ .

C. The procedure followed is as given in Instruction A except that the emulsifier added consists of 7.5 parts of a reaction product from 1 mol of diethylenetriamine and 2 mols of stearic acid, which reaction product is quaternised with dimethyl sulfate, and the soft-handle agent added consists of 75 parts of the acid amide of the formula given in Instruction B.

D. The procedure followed is as given in Instruction A except that the soft-handle agent added comprises 75 parts of the acid amide of the formula



wherein R<sub>5</sub> denotes

- 40 to 60% of  $-(\text{CH}_2)_{15}-\text{CH}_3$
- 20 to 40% of  $-(\text{CH}_2)_8-\text{CH}=\text{CH}-(\text{CH}_2)_7-\text{CH}_3$
- 10 to 20% of  $-(\text{CH}_2)_{17}-\text{CH}_3$
- 0 to 5% of  $-(\text{CH}_2)_{13}-\text{CH}_3$
- 0 to 5% of  $-(\text{CH}_2)_8-\text{CH}=\text{CH}-\text{CH}_2-\text{CH}=\text{CH}(\text{CH}_2)_4-\text{CH}_3$ .

E. The procedure followed is as given in Instruction A except that the soft-handle agent added consists of 75 parts of the acid amide of the formula



wherein R<sub>6</sub> denotes

- 60 to 70% of  $-(\text{CH}_2)_{21}-\text{CH}_3$
- 30 to 40% of  $-(\text{CH}_2)_{19}-\text{CH}_3$ .

F. The procedure followed is as given in Instruction A except that the soft-handle agent added consists of 75 parts of the acid amide of the formula



wherein R<sub>4</sub> has the meaning given in Instruction B.

G. The procedure followed is as given in Instruction A except that the soft-handle agent added consists of 75 parts of the acid amide of the formula



(13) 5

wherein  $\text{R}_7$  denotes

- 40 to 60% of  $-(\text{CH}_2)_8-\text{CH}=\text{CH}-(\text{CH}_2)_7-\text{CH}_3$
- 20 to 40% of  $-(\text{CH}_2)_{17}-\text{CH}_3$
- 10 to 20% of  $-(\text{CH}_2)_{15}-\text{CH}_3$
- 0 to 5% of  $-(\text{CH}_2)_{13}-\text{CH}_3$
- 0 to 5% of  $-(\text{CH}_2)_8-\text{CH}=\text{CH}-\text{CH}_2-\text{CH}-(\text{CH}_2)_4-\text{CH}_3$ .

10

H. The procedure followed is as given in Instruction A except that the soft-handle agent added consists of 75 parts of the acid amide of the formula given in Instruction B.

I. The procedure followed is as given in Instruction A except that the soft-handle agent added consists of 75 parts of the acid amide of the formula



(14)

wherein  $\text{R}_8$  denotes

- 30 to 50% of  $-(\text{CH}_2)_8-\text{CH}=\text{CH}-(\text{CH}_2)_7-\text{CH}_3$
- 20 to 30% of  $-(\text{CH}_2)_{17}-\text{CH}_3$
- 10 to 20% of  $-(\text{CH}_2)_{15}-\text{CH}_3$
- 5 to 15% of  $-(\text{CH}_2)_{13}-\text{CH}_3$
- 5 to 15% of  $-(\text{CH}_2)_8-\text{CH}=\text{CH}-\text{CH}_2-\text{CH}-(\text{CH}_2)_4-\text{CH}_3$ .

25

J. The procedure followed is as given in Instruction A except that the soft-handle agent added consists of 75 parts of the acid amide of the formula



(15) 35

wherein  $\text{R}_8$  has the meaning given in Instruction I.

K. The procedure followed is as given in Instruction A except that, for comparative purposes, no acid amide as soft-handle agent is added.

40

### EXAMPLE 1

A polyacrylonitrile yarn is treated for 20 minutes at 40° C. in the exhaust process, with a ratio of goods to liquor of 1:30, using an aqueous preparation of which the pH value has been adjusted to 5.5 with acetic acid and which contains, relative to the weight of the yarn, 2% of the dispersion according to Instruction A. To the dispersion is added before its application the 5-fold amount of water at 80° C.; the dispersion is then stirred and subsequently diluted with cold water, the pH value of which has been adjusted to 5.5 with acetic acid. After the exhaust operation, the yarn is dewatered without rinsing and is then dried at 60° C.

50

After drying and after conditioning at 20° C. with 40% relative humidity for 24 hours, the soft handle of the yarn is assessed, while 0 (no soft handle effect) representing the poorest rating and 4 (very good soft handle effect) the highest rating. In order to assess the fastness to fine-washing possessed by the soft-handle finish of the yarn, this is washed in a domestic washing machine for 30 minutes at 40° C. with a liquor containing per liter 2 g of a commercial fine detergent.

55

The yarn treated in this manner receives both before and after machine washing the rating 4 in the soft-han-

dle test, whereas the untreated yarn receives the rating 0.

### EXAMPLE 2

A polyacrylonitrile yarn is dyed, in a hank dyeing machine, in the exhaust process using a goods to liquor ratio of 1:35 with the dye liquors A and B of the following compositions, respectively, with a soft-handle finish being simultaneously imparted to the yarn.

#### Liquor A

0.28% of the yellow dye of the formula



0.14% of the red dye of the formula



0.35% of the blue dye of the formula



2% of 40% acetic acid (pH of the dye liquor: 4.5),  
1% of an alkylammonium salt as commercial leveling agent, and

2% of the dispersion according to Instruction A.

#### Liquor B

0.15% of the yellow dye of the formula



0.20% of the red dye of the formula



0.30% of the blue dye of the formula



2% of 40% acetic acid (pH of the dye liquor: 4.5),  
10% of Na<sub>2</sub>SO<sub>4</sub>·10H<sub>2</sub>O, and

2% of the dispersion according to Instruction A.

The dilution of the dispersion according to Instruction A is carried out as described in Example 1.

In the formulae (14) to (16), A<sup>⊖</sup> denotes an anion, for example



All percentages of the constituents of the liquors A and B are relative to the weight of yarn to be treated.

In dyeing by the so-called trichromic process, the yarn is immersed in the liquors A and B, respectively, at 60° C.; the yarn is then heated in the respective dye liquor, at a heating-up rate of 1° C. per minute, to 98° C., held for 60 minutes at this temperature, and after this period of time cooled again to 60° C. Without being rinsed, the dyed yarn is subsequently dewatered, and dried at 60° to 70° C. The yarns treated with the liquors A and B, respectively, receive the soft-handle rating 4. Furthermore, the presence of the dispersion according to Instruction A in the dye baths A and B has no retarding action on the employed dyes. There are obtained level grey dyeings having good depth of colour in the desired shade.

The yarns treated with the liquors A and B, respectively, according to Instruction A but without dispersion, as well as untreated yarn, are given the soft-handle rating 0.

### EXAMPLE 3

The procedure is performed in the manner described in Example 1 except that there is used an aqueous preparation containing 2% of the dispersion according to the following Table I instead of 2% of the dispersion according to Instruction A. The results of the soft-handle assessment, before and after washing with the fine detergent in the domestic washing machine, are likewise summarised in the following Table I.

TABLE I

| Emulsion used in the preparation                                    | Soft-handle test (ratings) |               |
|---------------------------------------------------------------------|----------------------------|---------------|
|                                                                     | before washing             | after washing |
| dispersion according to Instruction B                               | 4                          | 3.5           |
| dispersion according to Instruction C                               | 4                          | 3.5           |
| dispersion according to Instruction D                               | 4                          | 3.5           |
| dispersion according to Instruction E                               | 3.5                        | 3.5           |
| dispersion according to Instruction F                               | 3.5                        | 3.5           |
| emulsion according to Instruction K (contains no soft-handle agent) | 1.0                        | 0.5           |
| untreated yarn                                                      | 0                          | 0             |

Similar results are obtained with the dispersions according to Instructions G, H, I and J.

### EXAMPLE 4

5 A soft-handle finish is imparted, in separate baths in the exhaust process, to the following substrates: a cotton sponge cloth (CO), a woollen knitting yarn (WO), a crimp yarn made from polyamide (PA), a blended yarn made from wool and polyacrylonitrile (WO/PAC 10 50:50), a blended yarn made from wool and polyester (WO/PES 50:50), and a yarn made from a mixture of cotton and polyester (CO/PES 50:50). The treatment is carried out during 20 minutes at 40° C., with a ratio of goods to liquor of 1:30, using an aqueous preparation of which the pH value is adjusted to 5.5 with acetic acid, and which contains, relative to the weight of the material, 2% or 3% of the dispersion according to Instruction A, which has been diluted as described in Example 1. The cotton sponge cloth and the yarns and blended yarns mentioned in the foregoing are subsequently de-watered without being rinsed and are then dried at 60° C. The results of the soft-handle test after drying and conditioning are summarised in the following Table II. The untreated textile materials receive a handle rating of 0.

TABLE II

| Treated material | Amount of dispersion according to Instruction A | Soft handle rating |
|------------------|-------------------------------------------------|--------------------|
| CO               | 3%                                              | 4                  |
| WO               | 2%                                              | 3.5                |
| PA               | 2%                                              | 4                  |
| WO/PAC 50:50     | 3%                                              | 3.5                |
| WO/PES 50:50     | 3%                                              | 3                  |
| CO/PES 50:50     | 3%                                              | 3.5                |

### EXAMPLE 5

10 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 88

## EXAMPLE 8

2.5 kg of a polyacrylonitrile tricot is washed in a domestic washing machine (capacity: 5 kg of washing and 12 liters of water) is washed with an aqueous liquor at 40° C. containing 30 g of a commercial fine detergent. The water used has a hardness of 15° (German degree of hardness). After the fine detergent has been washed out, the tricot is treated with a final rinsing bath at room temperature containing 50 g of the dispersion according to Instruction A, which dispersion has previously been diluted as described in Example 1. After being rinsed, the tricot is centrifuged and then dried at 80° C. It is given the rating 4 in the soft-handle test, whereas a polyacrylonitrile tricot washed in the same manner but rinsed in the absence of the dispersion according to Instruction A is given the rating 0.

## EXAMPLE 9

The procedure is carried out as described in Example 8 except that 2.5 kg of a polyester knitted fabric is used instead of the polyacrylonitrile tricot. The tricot washed and rinsed according to the invention receives the rating 2.5 in the soft-handle test, whereas polyester fabric which has been similarly washed but rinsed in the absence of the dispersion according to Instruction A receives the rating 0.

## EXAMPLE 10

The procedure is carried out as described in Example 8 except that 2.5 kg of a polyamide knitted fabric is used in place of the polyacrylonitrile tricot. The knitted fabric washed and rinsed according to the invention receives the rating 3 in the soft-handle test, whereas polyamide knitted fabric which has been similarly washed but rinsed in the absence of the dispersion according to Instruction A receives the rating 0.

## EXAMPLE 11

The procedure is carried out as described in Example 8 except that 2.5 kg of a cotton sponge cloth is used in place of the polyacrylonitrile tricot. The sponge cloth washed and rinsed according to the invention receives the rating 3 in the soft-handle test, whereas cotton sponge cloth which has been washed but then rinsed in the absence of the dispersion according to Instruction A receives the rating 0.

What is claimed is:

1. A process for imparting to a textile material a soft handle, which process comprises immersing the material at 20° to 100° C. for 5 to 120 minutes in an aqueous preparation containing an acid amide of the formula



or a reaction product from acrylic or methacrylic acid, or an alkyl ester thereof, and an amine of the formula



wherein R<sub>1</sub> is alkyl or alkenyl of 14 to 22 carbon atoms and X is hydrogen or methyl, and subsequently drying the material at 50° to 150° C.

2. A process according to claim 1 in which there is used the acid amide of the formula



in which X is hydrogen or methyl.

3. A process according to claim 1 in which the preparation contains 0.1 to 0.5 percent by weight, relative to the dry textile material, of the acid amide or of the reaction product.

4. A process according to claim 1 in which the preparation is in the form of an aqueous emulsion or dispersion.

5. A process according to claim 1 in which the preparation contains, in addition to the acid amide or to the reaction product, 0.01 to 0.05 percent by weight, relative to the dry textile material, of an emulsifier.

6. A process according to claim 1 in which the preparation contains, in addition to the acid amide or to the reaction product and in addition to the emulsifier, 0 to 0.05 percent by weight, relative to the dry textile material, of a wetting agent.

7. A process according to claim 1 in which the preparation has a pH value of 4 to 6.

8. A process according to claim 1 in which the textile material consists of natural or synthetic fibers, or of mixtures of natural and synthetic fibers.

9. A process according to claim 1 in which the textile material contains wool, cotton, polyacrylonitrile, polyester or polyamide.

10. A concentrated composition for performing the process according to claim 1, which composition is in the form of an aqueous emulsion or dispersion which contains

10 to 50 percent by weight of the melted acid amide or of the reaction product,

0.1 to 5 percent by weight of an emulsifier, and  
0 to 5 percent by weight of a wetting agent.

11. A composition for performing the process according to claim 1, which has a pH value of 4 to 6 which is adjusted to the required value with a weak acid.

12. A composition for performing the process according to claim 1, which is obtained from a high-pressure emulsion and which at room temperature is in the form of a dispersion.

\* \* \* \* \*